

## UNITED STATES PATENT OFFICE

2,419,231

ELECTROPLATED CORROSION PROOF  
METAL ARTICLES AND METHOD OF  
MAKING THE SAMEDonald H. Schantz, Coraopolis, Pa., assignor to  
Standard Steel Spring Company, Coraopolis,  
Pa., a corporation of PennsylvaniaNo Drawing. Application December 21, 1940,  
Serial No. 371,100

9 Claims. (Cl. 29—191.6)

1

This invention relates to the protection of metals from attack by corrosive and similar reagents and has particular reference to the application of metallic coatings to the surfaces of the articles which are to be protected. Its main object is to provide effective coatings having many advantages over any prior coatings known to the applicant.

The protection afforded by applied metallic coatings arises mainly from the degree to which they are continuous or free from defects. Until recently, at least, it has been generally assumed by workers in the art that the protective value of metallic coatings also depends upon the position of the coating materials in the electro-chemical scale relative to the base metal. Lately, doubts have arisen whether that theory is a sound one, but it is used in this specification only as a convenient basis for explaining the invention. Nickel and copper, for example, are, according to the theory, electro-negative to iron and steel and depend upon continuity of coating for protecting the underlying metal. A break or defect in the coating of either of these metals, which exposes the iron, will not only permit but may actually accelerate corrosion of the underlying metal.

Zinc is electro-positive to iron and a zinc coating on iron or steel will give substantially complete protection if the coating is free from breaks or defects exposing the underlying metal. If there are breaks or defects in the zinc coating the underlying or base metal will not corrode or rust so long as there is zinc available on the surface of the article in the vicinity of a break or defect. It is difficult, if not impossible, to get a zinc coating in commercially practical thicknesses having perfect continuity, and, in addition, such coatings are subject to accidental damage. The electrolytic potential of zinc relative to iron is such that the consumption or dissolution of zinc when it starts to give way under corrosion is more rapid than is necessary for good protection, so that the effective life of the coating is shorter than it should be.

An object of the invention is to provide a method of applying a protective coating, which is singularly free from pores, pinholes and defects of a similar nature, and which is also of such a composition that it is not easily damaged.

Another object is to employ zinc for protective coating purposes, but in such a way that the difference in electrolytic potential between the coating and the metal base is reduced to a point intermediate that of zinc and iron. This result

2

is accomplished by coating the surface of the article with an alloy of nickel and zinc which is less anodic to iron or steel than zinc, thereby slowing down the decomposition of the coating in the case of a break or defect through which harmful agents might penetrate to set up electrolytic action.

Still another object is to make it possible to electroplate alloys of nickel and zinc on a commercial basis. This has not previously been done successfully. This is done by employing a new buffered electrolyte, high in metal content, and using quite high current densities. The preferred range of density is from 300 to 700 amperes per square foot of cathode area, although densities below and above the ones specifically mentioned may be used. The invention further includes new correlations of temperature, pH or hydrogen ion concentration, and buffer concentration, which may be varied to control the percentages of nickel and zinc in the alloy deposited.

Microscopic examination of a typical nickel-zinc alloy, formed by heating the two metals while in contact, shows that the alloy has a stratified appearance and analysis shows that the nickel and zinc, in what are for convenience termed the strata or layers of alloy, conforms in structure to the nickel-zinc alloy system as follows:

|    |                |              |
|----|----------------|--------------|
| 30 | Alpha          | Up to 28% Zn |
|    | Beta (sub-one) | 50-44% Ni    |
|    | Gamma prime    | 24-20% Ni    |
|    | Gamma          | 20-13% Ni    |
|    | Delta          | 12-10% Ni    |

35 Successively stripping off the different strata or layers and corrosion tests after each strata has been removed indicate that the gamma layer is the most effective part of the alloy structure from a corrosion resisting standpoint.

It is not clear why the gamma alloy on steel possesses a better corrosion resistance than zinc on steel. However, some tests have indicated a provisional or working hypothesis. When the 40 gamma alloy is immersed in a corroding solution its potential with respect to the solution is only slightly less electro-negative than that of zinc immersed in the same solution. When, however, gamma is coupled to iron and the potential of the couple is measured, the resulting value is the same as that obtained for iron alone; when zinc is coupled to iron, the potential of the combination is that of zinc. It may be stated from this

45 that the gamma-iron couple is under "anode control"—i. e., the area of the anode (gamma) con-

trols the rate of corrosion. For the zinc-iron combination, the couple is under "cathode control"—i. e., the area of the cathode (steel) controls the corrosion rate. Thus for zinc coated steel, as any pore in the zinc coat is enlarged by corrosion, the area of the cathode increases considerably, and the corrosion rate correspondingly increases. As a pore in gamma-coated steel is enlarged, the anode area is not changed much, and therefore the corrosion rate remains constant. This may in part be due to the physical structure of the gamma alloy, or it may be due in part to the fact that the gamma alloy has greater continuity, or it may be almost entirely due to the fact that the gamma alloy is only slightly electro-positive to iron or steel. While, as stated, the gamma alloy seems to be the best from the standpoint of protection, the gamma prime and delta alloys are effective, but to a lesser extent than the gamma alloy. In fact, nickel-zinc alloys having an amount of nickel less than the amount found in the delta alloy give worthwhile results. Apparently, however, pronounced benefit from the nickel-zinc alloys is found only when the percentage of nickel is somewhere between about 3 percent and about 24 percent, with about 11 to 18 percent giving best results.

By this invention a nickel-zinc alloy is deposited from a single electrolyte and in the proportions of nickel and zinc desired. In the best practice the percentage of nickel is kept within the limits of 11 to 18 percent nickel and the rest zinc. This result can readily be obtained by using electrolytes such as are hereinafter specified, having a high metal content and effecting deposition of the metals simultaneously by using a high current density.

A bath or electrolyte which is representative, contains, to the gallon, thirty-five ounces of zinc sulphate calculated as  $ZnSO_4 \cdot 7H_2O$  or about 16.7 ounces of zinc chloride  $ZnCl_2$ . The zinc metal content should be from about seven to about nine ounces. Nickel is introduced as a chloride. About eight ounces of nickel metal should be introduced by adding to the electrolyte about thirty-two ounces of  $NiCl_2 \cdot 6H_2O$ . The electrolyte also contains a buffer which may be acetic acid, formic acid or citric acid at a concentration of about .5 normal. The salts of some of these acids may be used. This buffered electrolyte may have, in operation, a pH of from about 1 to about 3, but a pH of from 1.5 to 2.5 is preferred. The pH may be adjusted by using hydrochloric acid to lower it, and either nickel or zinc carbonate or zinc oxide to raise it. The electrolyte should be kept in circulation in a well known manner when the articles being plated are simply suspended in the electrolyte, but in plating continuously upon wire or strip moving through the electrolyte such circulation may not be necessary.

It is preferred to use separate nickel and zinc anodes having their surface areas relatively proportioned on the same ratio as the nickel and zinc in the desired alloy. In order to get the right distribution of the current to the cathode, the article which is receiving the deposit, it is preferred to use a plurality of zinc anodes and a plurality of nickel anodes and so position them on the anode support as to get the current distribution desired.

Instead of using separate zinc and nickel anodes, cast or rolled alloy anodes having the metals in about the same proportions as in the alloy being plated out may be used; or nickel anodes may be used and the zinc salt added as necessary

to replace the zinc plated out; or zinc anodes may be used and the nickel replenished by adding nickel salts. Insoluble anodes may also be used, but this requires constantly adding both the zinc and the nickel salts to replace the metals which have been plated out.

The operating temperature for an electrolyte made up as above directed may be from 70° to 150° F., a temperature of 125° F. giving good results in plating an alloy containing 11 percent to 18 percent nickel.

The current generators employed are of the usual type, the voltages running from 6 to 24 volts, depending both upon the distance from the anode to the cathode and the amperage desired. For coating sheets and strip about 300 amperes to the square foot of cathode surface appears to be best, regardless of whether the material is suspended in the electrolyte or is fed continuously through the electrolyte. Wire can be plated at about the same amperage per square foot as is mentioned for sheets and strip, but better results commercially are obtained in the continuous plating of wire if the current density is 500 amperes or higher per square foot of cathode surface. It is important in all instances that the current density selected for a particular alloy plating operation shall be kept uniform.

The electrolyte constituted as above specified, and the preferred arrangement of zinc anodes and nickel anodes receiving a current adjusted to about 300 amperes per square foot of cathode surface, will simultaneously deposit on the cathode a nickel-zinc alloy in which the zinc and nickel will be present in percentages averaging approximately 85 percent zinc and 15 percent nickel.

The percentage of zinc in the alloy may be controlled by raising and lowering the pH of the electrolyte, by raising or lowering the amperage within definite limits, by changing the temperature of the electrolyte, by the use of zinc sulphate instead of zinc chloride when the lower percentages of nickel are desired, by regulating the degree of agitation or rate of circulation of the electrolyte, and by changes in the relative amounts of zinc and nickel in the electrolyte. Such changes are a matter of experience with particular products. The total metal content to the gallon of electrolyte should, however, generally be at least fourteen ounces for the best results with high current densities.

The following are some examples illustrating changes in the procedure to get a desired percentage of nickel and zinc in the alloy.

For continuous plating of the alloy on a wire, a solution has been employed which contained 8½ ounces of nickel metal (about 35 ounces  $NiCl_2 \cdot 6H_2O$ ), 10 ounces of zinc metal (about 2½ ounces  $ZnCl_2$ ), and acetic acid 3 percent by volume. The pH of the solution was adjusted at 2.2 and the temperature of the solution was raised to 124° F. with the wire traveling at seven and one-half feet per minute through the solution, a current of 515 amperes per square foot of cathode area deposited on the wire a coating of alloy containing 14 percent nickel and the remainder zinc.

Sheets suspended in an electrolyte in which the nickel metal was 7.2 ounces to the gallon and the zinc 8.5 ounces to the gallon and which had a temperature of 115° F. and a pH of 2.3 deposited 10 percent nickel and 90 percent zinc when a current density of 100 amperes per square foot of cathode surface was employed. The zinc was introduced in sulphate form.

When the electrolyte was made up to contain 8 ounces of nickel metal and 7.4 ounces of zinc metal to the gallon, with the pH adjusted to 2.3 and the temperature to 125° F., the percentage of nickel deposited by a current of 300 amperes per square foot of cathode surface was approximately 15 percent.  $ZnSO_4 \cdot 7H_2O$  was used instead of  $ZnCl_2$ .

An electrolyte containing 8.4 ounces of nickel and 7.0 ounces of zinc (introduced in sulphate form) to the gallon with a pH of 2.4 deposited 20 percent nickel when the current density of 400 amperes per square foot cathode surface was employed and the temperature of the electrolyte raised to 145° F.

In all of the examples just mentioned the nickel was introduced as a chloride and the buffer was acetic acid.

The alloy may be plated directly upon the metal article after the surface thereof has been properly cleaned, and the alloy coating so deposited is adherent, continuous and protective to pronounced degrees. It is preferred, however, to first deposit upon the surface of the article a primary coating of copper or nickel (nickel is preferred) from 0.000025" to 0.000100" thick. Nickel is in itself a protection against corrosion if continuous and, in addition, being electro-negative to steel, it probably at least slows down the electrolytic action between the anodic alloy and the base metal where the latter is exposed.

The nickel plated article is next rinsed and then given a coat of alloy plating from the nickel-zinc electrolyte. The thickness of the alloy coating may vary within a wide range, being dependent upon the environment in which the article is to be used. Usually a thickness of 0.000300" is ample for protection against all except very severe conditions.

While in the foregoing the base metal to be protected has usually been referred to as iron or steel, the electrolyte and method of alloy plating can be employed without substantial change on many non-ferrous metals and metal alloys in the form of sheets, strip or wire.

Also in the foregoing, reference has been made to sheets, strip and wire, but the electrolyte and method of depositing it can also be used without change in protecting other mill products and fabricated articles, for example, tubing and woven wire products. Here again it is preferred to first coat such products with a thin coating of nickel, a thickness of from 0.000025" to 0.000050" being sufficient, after which the alloy coating is deposited. This latter coating may be of any desired thickness but from 0.000200" to 0.000300" is ample for all ordinary requirements.

Articles which have been corrosion proofed according to this invention have shown no signs of corrosion of the base metal after having been subjected to the standard salt spray tests for hundreds of hours. The process is a simple one to follow and the resulting product is better from a corrosion-resistant standpoint than anything found in the prior art, with many other advantages present which are not found in products resulting from any prior practice. The equipment necessary is, of course, more or less standard in the plating art.

In explaining the invention, various examples have been given, but it is apparent that they were illustrative only. It is obvious that the invention can be employed in other ways, to produce various products, all coming within the claims which follow.

What is claimed is:

1. The method of plating articles with a nickel-zinc alloy which includes making the articles cathode in an electrolyte, having a pH between about 1 and about 3, in which nickel chloride and zinc salt of the group consisting of zinc sulphate and zinc chloride have been dissolved in sufficient amounts to give, to each gallon of the electrolyte, a metal zinc content of about 7 to 9 ounces and a nickel metal content of about 7 to 8 ounces, and passing a current having a density of 100 to 700 amperes to the square foot of cathode surface through the electrolyte to the articles.
2. The method of plating articles with a nickel-zinc alloy which includes making the articles cathode in an electrolyte consisting of, to the gallon of water, about 17 ounces of zinc chloride, about 32 ounces of nickel chloride and about 3 percent by weight of a buffer selected from the group consisting of acetic, citric and formic acids, and passing through the electrolyte to the cathodes a current of from about 100 to about 700 amperes per square foot of cathode area, the amperage and the time during which the article is in the electrolyte depending upon the percentage of nickel and zinc and thickness of deposit desired.
3. A ferrous metal article having an adherent protective coating consisting of a layer of electro-deposited nickel, and an outermost exposed alloy layer at least as thick as the nickel layer consisting of nickel and zinc simultaneously deposited on the nickel layer from a single electrolyte and containing an average of about 15 percent nickel.
4. A ferrous metal article having an adherent protective coating consisting of a layer of electro-deposited nickel, and an outermost exposed layer at least as thick as the nickel layer consisting of nickel and zinc simultaneously deposited from a single electrolyte and containing from about 10 percent to about 24 percent nickel and the rest zinc.
5. A plating solution having a pH of over about 1.0 and under about 3.0 containing, to the gallon of solution, about thirty-five ounces of zinc sulphate, about thirty-two ounces of nickel chloride, and about 3 percent by volume of a buffer of the group consisting of acetic acid, formic acid, citric acid, and salts thereof, the rest of the solution being water.
6. A plating solution having a pH between about 1.0 and about 3.0 containing, to the gallon, about 16.7 ounces of zinc chloride, about thirty-two ounces of nickel chloride, and about 3 percent by volume of a buffer of the group consisting of acetic acid, formic acid, citric acid, and salts thereof, the rest of the solution being water.
7. A plating solution containing to the gallon of solution, about thirty-five ounces of zinc sulphate, about thirty-two ounces of nickel chloride, about 3 percent by volume of a buffer of the group consisting of acetic acid, formic acid, citric acid, and salts thereof, and addition agents adjusting the pH to about 2.5, the rest of the solution being water.
8. A plating solution having a pH of over about 1.0 and under about 3.0 containing, to the gallon of solution, a salt of the group consisting of zinc sulphate and zinc chloride in amount to give about 7 to 9 ounces of zinc, nickel chloride to give about 7 to 9 ounces of nickel, and a buffering agent of the group consisting of acetic acid, formic acid, citric acid, and salts thereof, the rest of the solution being water.

9. The method of plating articles with a nickel-zinc alloy which includes making the articles cathode in an electrolyte containing material of the group consisting of acetic acid, formic acid, citric acid and salts thereof, having a pH between about 1 and about 3 and a temperature between about 100° F. and about 150° F., and consisting substantially of zinc salt of the group consisting of zinc sulphate and zinc chloride in amount to give about 7 to 9 ounces of zinc metal to the gallon, and nickel chloride in amount to give about 7 to 8 ounces of nickel metal to the gallon, and plating nickel and zinc simultaneously on the cathode by passing a current of over 100 amperes and under 1,000 amperes to the square foot of cathode through the electrolyte to the cathode.

DONALD H. SCHANTZ.

5

10

15

## REFERENCES CITED

The following references are of record in the file of this patent:

## UNITED STATES PATENTS

| Number    | Name          | Date         |
|-----------|---------------|--------------|
| 1,564,581 | Schoch et al. | 1907         |
|           | King          | Dec. 8, 1925 |

## OTHER REFERENCES

Transactions of the Electrochemical Society, vol. XI (1907), Schock et al., pp. 136-139. (Copy in Div. 36.)

Trans. Electrochem. Soc., vol. 73 (1938), pp. 417-433. (Copy in Div. 56.)